

April 23, 1946.

R. F. WARREN, JR.

2,399,157

## ROPE

Filed June 19, 1940



Fig. 1



132 Fig. 2



Fig. 5



Fig. 6



Fig. 3

Fig. 4

INVENTOR.  
RICHARD F. WARREN JR.  
BY *John F. Hanahan*  
ATTORNEY.

## UNITED STATES PATENT OFFICE

2,399,157

## ROPE

Richard F. Warren, Jr., Stratford, Conn.

Application June 19, 1940, Serial No. 341,352

11 Claims. (Cl. 57—147)

This invention relates to new and useful improvements in ropes.

The objects and advantages of the invention will become apparent from a consideration of the following detailed description taken in connection with the accompanying drawing wherein satisfactory embodiments of the invention are shown. However it is to be understood that the invention is not limited to the details disclosed but includes all such variations and modifications as fall within the spirit of the invention and the scope of the appended claims.

In the drawing:

Fig. 1 is a side elevational view of a short section of the rope of the invention a portion of the outer strands being broken away and part of the core being shown as never having had the outer strands laid about the same;

Fig. 2 is a somewhat enlarged transverse sectional view taken as along the line 2—2 of Fig. 1;

Fig. 3 is a perspective view showing a rope core alone;

Fig. 4 is a view somewhat similar to Fig. 3 but showing another modification of the rope core;

Fig. 5 is an enlarged transverse sectional view showing a modification of rope; and

Fig. 6 is a view similar to Fig. 5 but showing another modification of rope.

Referring in detail to the drawing and at first more particularly to Figs. 1 and 2 at 127 is shown a rope including a main core 128 over which are laid strands 129 each comprising a core 131 and a series of wires 132 laid or twisted over such core. Strands 129 are circular in transverse section although the invention is not limited to such construction. For use in drag lines and the like other shapes of strands and elements may be employed as, for example, wedge or triangular shaped strands and elements may be used. The main core 128 is a bar-like filament and prior to incorporation in the cable is of constant diameter and round in transverse section. As will later develop, this core is extruded. Core 128 and cores 131 are of plastic, preferably vinylidene chloride.

The strands 129 are laid about the main core 128 under tension whereby portions of the wires 132 coming into contact with such core deform it providing grooves 133 shown in Fig. 1. The core is resilient whereby as the rope is put under tension the rope strands may further deform the core but as the load eases the core will tend to return to its original shape. Since the core is round it is engaged the same on all sides by the strands 129

whereby such strands are uniformly supported throughout the length of the rope.

Fig. 3 shows a core separate from any other rope structure. This core generally designated 131, comprises a plurality of small diameter vinylidene chloride filaments 138 twisted together. Core 131 is quite flexible and provides considerable surface area for the application of lubricant.

Core 131 has many desirable characteristics and particularly where it is made of a large number of relatively small diameter filaments it is substantially circular in transverse section and provides a uniform support for strands laid about it. However the core is but loosely twisted and care should be taken in unreeling it so that it does not untwist whereby it may be kept with the foreheart originally laid into it.

Fig. 4 shows a construction wherein the vinylidene chloride, of which the core generally designated 144 is formed, has first been cut or formed into strips. Thereafter the strips are twisted to provide filaments 145 and any desired number of these are twisted together to provide the core. A core made by the twisting up of a single strip 25 of the material may be used. However, for larger or main cores a plurality of strips are twisted together to provide the core with the desired solid characteristics and with the desired resiliency and elasticity.

Fig. 5 shows a rope including fillers 173. In such figure the rope is generally designated 174 and the same includes a number of strands designated respectively 175, 176, 177, 178, 179 and 180 each made up of a number of wires or metallic elements. The strands are arranged about a central core 181 which may be of hemp or other natural fibres or of any of the plastics, the characteristics of which have been set forth. In fact the core may be of metal strands if so desired and if of plastic, may be any of the constructions of cores heretofore considered.

Each of the strands of the present rope is made up of a number of metallic elements or wires 182 and of a number of smaller diameter metallic elements 183 (of which five are shown) and of the fillers 173 of vinylidene chloride. At the center of each strand is an element 184 of metal or of plastic.

The rope 174 is much more flexible than it would be if the filler elements 173 were of metal. These elements do not add particularly to the tensile strength of the rope but they do serve to prevent the metal elements thereof from nicking one another and act as cushions for such elements. Additionally when loaded with lubri-

cant as they may well be, the fillers 173 serve to retain the lubricant and free it as may be required during use of the rope as disclosed in my copending application.

Fig. 6 shows a Seale type rope generally designated 185 and comprising six strands 186, 187, 188, 189, 190 and 191 arranged about a main central core 192 of natural fibres or of the construction of any of the cores 137 and 144 above mentioned. Each strand of rope 185 comprises a plurality of wires or metal elements 193 arranged in a circle about and in spaced relation to a central metal element 194 and about said central element and between it and the larger outer wires 193 is a ring of vinylidene chloride filaments 195. These plastic filaments do not make for a rope or cable having the tensile strength of a rope or cable wherein the mentioned elements are of steel, but have more strength than if natural fibre is used.

The plastic filaments make for a rope or cable of great flexibility and in addition the plastic filaments act as cushions preventing nicking of the inner and outer metal elements on one another. As the rope is laid and as it is used, the various stresses set up in it will result in deformation of the plastic filaments from the precise form in which they are shown but the plastic material will be present between the inner and outer metallic elements to function as a cushion and when loaded with lubricant will serve to retain and feed the latter as it may be needed during use of the rope.

In making the rope of the invention each of the filaments (metallic and non-metallic) is preformed or formed on a helix whereby the filaments in a strand interfit with one another without stress. Thus should any filament become broken the ends of such filament will not have a tendency to spread outwardly of the zone of the body of the strand and will resist unstranding and thus remain in place giving something to the strength of the assembly. This same preforming operation is carried out in connection with the strands made of the preformed filaments whereby the strands being formed into helices will lie in an unstressed neutral condition in the ropes.

The preformed construction has little internal stress and therefore, ropes made as described will lie in a flat or straight condition with no real tendency to snarl or twist. When the ropes are to be cut it is not necessary to seize the ends as they will not unlay. Also such ropes have a longer life when run on sheaves; they are easier to splice; resist rotating in grooves; spool or coil perfectly and resist whipping.

While in connection with the disclosed embodiments of the invention the various non-metallic filaments and cores have been described as of vinylidene chloride it is to be understood that such material is the plastic preferred in the making of my ropes but that other plastic may be used. Generally speaking the non-metallic filaments or cores comprise organic plastic materials or certain inorganic natural plastic materials as glass fibres, quartz fibres, or Bentonite (in the form known as Alsifilm) although asbestos has been found useful for my present purpose.

In fact some of the organic plastics may be used with clay or other cheap fillers as well as with fillers of cotton, silk, wool, waste ends from rope making, or other fibrous materials both natural and synthetic. Thus cotton, silk, wool, rayon

and other regenerated celluloses, or other fibrous material may be used in the form of flock, stable fibres, threads, swatches of woven fabrics or impregnated sheets cut to strips for twisting into elements or strands. In addition cellulose derivatives while in alpha and beta stage may be used as fillers and to toughen the material.

Vinylidene chloride possesses about all of the characteristics required. It is oil, acid, and alkali resistant, non-inflammable, has the desired modulus of elasticity, tensile, abrasive and flexural strength, is resilient, will not oxidize, is not adversely affected by sun or other light rays and has exceptionally few solvents. Further it is for the most part (as are the other vinyl derivatives) resistant to corrosive halides such as chlorine and bromine and also to mustard gas. Vinylidene chloride is permanently water proof and is not affected by bacteria and will not support fungus growth and so is not likely to decay through biochemical attack. The vinylidene chloride (sold commercially as Venalloy) is in most respects mentioned herein similar to another vinyl compound sold commercially as Vinyon. However the latter is not as desirable due to the necessary use of plasticizers which dissipate in time making the material very brittle.

Vinylidene chloride has a critical point of set in that such material when stretched to the point of most yield has a return of about 10 percent. The stretching must be accomplished within a short time following extrusion as otherwise the material must be soaked in heat to cause it to return to random orientation to prevent the formation of cracks in its surface. Plastic filaments having a fixed amount of stretch and return provide a rope which gradually takes up its load. Where such filaments are used in a rope also having metal elements the feature of stretch is present since the metal elements may straighten and squeeze into the plastic filaments providing for elongation of the rope. The parts will return to normal on being relieved of the load. The initial portion of the stretch is most easily obtained and as the rope elongates each succeeding degree of elongation requires a greater or increased load so that the load in any given instance is gradually taken up.

The non-metallic filaments, and cores of the rope of the invention may be of any of the various plastics as above suggested and such plastics include synthetic resins, natural and synthetic latices, cellulose (as ethyl cellulose) and its derivatives, protein plastic substances (as nylon), and petroleum plastic derivatives. There are several chemical types of synthetic resins such as (1) phenol-aldehydic resins, (2) amino-aldehydic resins, (3) hydroxycarboxylic resins, (4) sulphonamide resins, (5) resins from sugar, (6) vinyl resins including resins from vinyl derivatives, (7) indene resins and (8) lignin plastic substances. The polymerization resins and particularly the vinyl resins including resins from vinyl derivatives are preferred for my purpose.

Under the type (1) may be included resins such as phenol formaldehyde, cresol and cresylic acid, other tar acids and formaldehydes, phenol furfuraldehyde or other tar acids and other aldehydes. Under type (2) is included urea and formaldehyde resins, and aniline resins obtained by condensing aniline and formaldehyde and other anilines or amines and other aldehydes.

Under type (3) I include materials produced by the esterification of polybasic acids with poly-

hydric alcohols. Such materials are frequently called alkyd resins, this title including adipic acids resins obtained by the condensation of adipic acid and glycerin or by the condensation of glycerin with phthalic anhydride. Type (4) includes the sulphonamide resins developed from para tolensulphonamide. The resins from sugar, type (5) above, are obtained by condensing saccharide with aldehydes and urea.

Vinylidene chloride (sold commercially as Venalloy) is included in the group of vinyl resins (type 6) including resins from vinyl derivatives and such group also comprehends vinyl ester, vinyl butyrate, vinyl chloride, acrylic resins from vinylcarbonylic acid ester, vinyl carbonylic acid, vinyl benzole or polystyrol, divinyl or butadiene, vinyl ester or vinyl chloride, copolymerized polyvinyl chloride and polyvinyl acetate (known commercially as Vinylite), vinyl acetate, polymers of vinyl halides combined with different percentages of plasticizers (known commercially as Koroseal) the commercial article known as Vistanex and comprising polyiso butylene polymerized with boron trifluoride and also comprising polyiso butadiene having a tacky to rubber-like structure, the commercial products known as Vynon (a copolymer of polyvinyl chloride and polyvinyl acetate), Butacite (a reaction product of vinyl acetate resin with butyraldehyde), and Rezel (resulting from the fact that the introduction of an unsaturated resinous ester of the maleate polyester type into a compound of the type



has the property of curing the latter), the polymer of ester of acrylic acid known commercially as Plexigum, polymers of the esters of methacrylic acids such as the polymethacrylic resin sold as Lucite and Plexiglas. Isobutyl methacrylic resins, certain plastic obtained by mixing the monomer of styrene with vinylidene chloride and with ethylene glycol and maleic acid and copolymerizing the mixture, styrene and in addition thereto the resin known as polystyrene.

Resins of the indene group (type 7) include polyindene and poly-cumaron. Under type (8) I include lignin and its derivatives extracted from paper mill waste waters and other sources. The lignin may be separated into various chemical components of no value to me here but also into colored gums and by various treatments into clear transparent resins useful for my present purpose. Lignin is hydrogenated with Raney nickel catalyst, in aqueous solution yielding methanol, propylcyclohexane, hydroxy propylcyclohexanes, and a colorless resin which may again be separated into an alkali soluble in an alkali insoluble component. I use either of these components in the production of resins to be used in the making of ropes.

Under the heading of natural and synthetic lastics, I include as natural lastics—Balata, rubber, gutta percha and latex to be used alone or as a coating or processed or compounded with other materials. As the synthetic lastics I mention polymerized chloroprene (of the type now sold as neoprene); polymerized butadiene (of the type sold as Buna or Perbunan); polymethylene polysulphide (of the type sold as Thiokol) chlorinated rubber (of the type sold as Tornesit); rubber hydrochloride (of the type sold as Pliofilm); and isomerized rubber (of the type sold as Pliform) and any latex of these. Also sulphonated rubber or synthetic sulphonates to promote wire adhesion.

Certain materials sometimes called synthetic lastics I prefer to include under the heading of vinyl derivatives. For example, it appears that the polymerized vinyl derivative known commercially as Vistanex (polyiso butylene and polyiso butadiene) might be included under either group. Such material is used in the present instance when mixed with other materials and has certain lubricating properties of value in the making of ropes.

Under the heading of cellulose and its derivatives I include cellulose acetate; regenerated cellulose; cellulose xanthate; benzylcellulose; ethylcellulose; cellulose hydrate; cellulose triacetate; cellulose acetobutyrate; cellulose acetopropionate; hydrolysed cellulose acetate and others of the cellulose esters and ethers. Rialan a rayon thread made from cellulose extracted from sugar cane may also be used. Most of these materials can be used alone for my purpose in the making of ropes and can be used in the form of filaments or may be cut to strips from sheets and then the strips twisted into filaments, such as those shown at 145 of Fig. 4. Also certain of these materials may be used with other materials herein mentioned for the purpose of toughening the latter.

Nitrocellulose compounded with other materials of a less flammable nature or of a nature to prevent flammability, may be used. Halowax or the like may be used for compounding with nitrocellulose and it is noted that the latter in so far as cost, strength and the like are concerned, is a desirable material for my purpose. Other non-inflammable plasticizers which may be compounded with nitrocellulose for my purpose are monophenyl phosphate and di (paratertiary butyl phenyl) mono 15 tertiary butyl 2 xenyl phosphate. The flammable nature of nitrocellulose may be weakened or lessened by mixing with varying proportions of cellulose acetate. Under this class may also be included gel cellulose which may be used for my purpose. This material may be used as a filler with other materials herein mentioned.

Under the heading of protein plastic substances, I include casein preferably in the fibrous form sold as Lactofil and Lanital made by either the wet or dry process. The material sold as Zein, and which comprises a raw material in the form of a powder, may be extrusion or the like be converted into fibres for use here. Polypentamethylene sebacamide sold as nylon may also be used. Regenerated silk made by reducing waste silk and waste cocoons containing silk and then forming it into threads or sheets to be cut to strips, is also believed to fall under the present heading.

That group of compounds of which at least one is obtained by condensation polymerization from a diamine and a dibasic carboxylic acid and of which one is now sold under the trade-mark Exton is very useful for my present purpose.

Another protein plastic which may be used is obtained by extracting the protein from the refuse remaining after the oil has been extracted from soy beans, oiticica nuts, and other protein bearing substances. The extracted protein is properly reacted to form plastic substances. Here it is noted that oiticica oil may be used as a plasticizer with styrene to make the latter more suitable for my purpose.

Collagen plastics are another protein substance suitable for my purpose. Such plastics are fibrous. The collagen may be recovered from the

waste from tanneries or otherwise. Various resins from coffee may also be used.

The petroleum plastic derivatives include those gums or resins obtained by the oxidation or controlled polymerization of certain distillates of petroleum cracking. Thus I may use the commercially known "Santoresins" produced by this method as well as "Petropol" which is a softer type of the same material. These materials are, when used for my purpose, to be mixed with other materials listed above whereby the resultant mass may be shaped by extruding or the like to provide threads or sheets of materials having desired characteristics. Propane precipitated resins from distillation of crude petroleum may also be used to advantage as an assistant to produce heat penetration to materials like vinylidene chloride and retain stability.

Also cracking coal tar resins of high aromatic content condensed with formaldehyde or other aldehydes forms resins useful for my purpose. Similarly, I may use heavier petroleum products cracked and then condensed with formaldehyde or other aldehydes, hydrogenated or chlorinated either at elevated temperatures or by the addition of metallic halides. For use as rope cores comprising large diameter bars and the like, the materials are advantageous. The natural inorganic materials above mentioned may be used in the place of the organic plastics in certain instances. The glass or the quartz must be made plastic by heat and then it is spun or extruded in fibres and the latter are oriented and brought together to form strands or cores as the case may be.

Plastics comprising nitrogenous condensation products are also suitable for use in the making of various rope elements of the invention. One such plastic is now on the market under the name "Nulamine."

Preferably when glass, fused quartz or other materials which may be made into fibres of great tensile strength are used as a material in the making of ropes, it is incorporated into strands or cores or other elements and such elements may be either solid one piece structures or they may be made up of a number of separate elements. The filaments, strands or cores comprise a plastic or a combination of plastics having the inorganic fibres embedded therein and oriented to extend in the direction of the length of the strands or cores.

Thus, in such a construction the glass or quartz fibres to as large an extent as possible or as is feasible, are oriented and also each fibre coated with a plastic or are otherwise spaced by the use of a plastic so that the fibres are maintained from contact with one another. The fibres are oriented. The presence of these oriented fibres very greatly increases the tensile strength of the filaments or cores and thus of the ropes into which they may be incorporated.

Bentonite, in especially pure form, may be mixed with water to form a gel. The gel is evaporated and the particles draw toward one another and become permanently fixed, by their attraction for one another, in strings or tiny fibrils. These mat together to form a tough coherent film. The bentonite may be extruded in the form of filaments or after being formed into sheets may be cut into strips and the latter twisted into filaments, such filaments to be used as above in the formation of strands or cores. Stressing of these gels produces orientation desirable for strength.

Under the general heading of asbestos, I include the fibrous varieties of the mineral amphibole,

the fibrous forms of pyroxene, the mineral crocidolite of the amphibole group and also chrysotile. The principal varieties of asbestos are anthophyllite, amphibole and serpentine. Asbestos floats of any variety may be used as fillers while the longer fibres may be made into filaments for strands or cores.

Various combinations of the materials disclosed may be used for the purpose of regulating real-  
10 iency, stiffness, bacteria growth, fungus growth, water-proofness, controlling the melting or soft-  
15 ening point, control of strength factors, as elas-  
ticity, tensile and shear strength, aiding in lubri-  
cation and the like. Many of the materials dis-  
16 closed herein and which are chemically incom-  
patible with one another are mechanically mis-  
18 cible to form a homogeneous mass adapted to be  
20 fabricated into filaments or bars, sheets and  
strips to be made into ropes, or cores meeting any  
22 of the above requirements as to combinations of  
24 physical and chemical characteristics. Thus ma-  
26 terials which may not be used alone for my pur-  
28 poses by reason of being too brittle and the like  
30 may be mixed with other materials and in that  
32 way utilized for the characteristics they may im-  
34 part.

Formaldehyde and urea resins as well as any  
36 chlorinated material (certain synthetic lastics),  
38 and the like have germicidal properties and when  
40 used with other materials included herein will  
42 serve to prevent or arrest bacteria growth and  
44 thus decomposition of the filaments or cores due  
46 to the action of bacteria or fungus. Whether the  
48 action of said materials merely arrests bacteria  
50 growth or completely eliminates bacteria will de-  
52 pend on the materials and the quantities used in  
54 the mixtures.

The various filaments (whether bundles of fine  
56 filaments or single bar-like elements of consid-  
58 erable diameter are employed) are oriented.  
60 Where preformed structures are employed it is  
62 preferred that the molecules of the filaments be  
64 oriented in a direction parallel to the axial cen-  
66 ters of the filaments. That is, the molecules are  
68 oriented in a direction parallel to the center of a  
70 helical line (the longitudinal center line of the  
72 filaments) rather than the parallel relation to a  
74 straight line. This is accomplished by stretch-  
76 ing the material through a helical die. Thus in  
78 my preformed strands or filaments I avoid obsti-  
80 nate internal stresses which cause a wildness of  
82 fibre. The strands, cores or ropes made of the  
84 filaments oriented as described will have in-  
86 creased tensile strength and extra resistance to  
88 twisting and bending, and will lay in a rope with-  
90 out opposing stresses tending to open the rope.

In orienting the filaments (whether thread-like  
92 or bar-like) they are reduced to the desired di-  
94 ameters by repeated small reductions obtained  
96 by drawing through successively smaller dies or  
98 by repeated stretching. Such reductions take  
100 place while the material is in a ductile condition.  
The preforming and orienting operations may be  
102 simultaneously accomplished.

In making the filaments of twisted strips 104 rather than by extrusion the sheets from which  
106 the strips are to be taken are reduced to the de-  
108 sired thickness by repeated small reductions  
110 rather than by a single large reduction. These  
112 reductions take place while the material is heated  
114 or wetted (depending on the material being used).  
116 The finished sheets are cut to strips and the lat-  
118 ter twisted into filaments for use in cores or the  
120 like.

122 Preferably the strips are cut from the sheet in

such manner as to have the direction of the length of the flow of the material of the sheet represent the longitudinal axis of the strips. Thereafter as the strips are twisted they are heated or wetted (depending on the material concerned) and are stretched whereby to further orient the molecules to have the latter oriented in the direction of the length of the twisted strip and on a bias with respect to that which was the longitudinal axis of the strip prior to the twisting thereof.

Having thus set forth the nature of my invention, what I claim is:

1. In a cable or rope, a strand comprising inner and outer metal elements, said elements transversely circular and all of substantially the same diameter whereby in the assembled strand there are longitudinally extending spaces, and smaller diameter longitudinally extending filler elements in said spaces and tangentially engaging both the inner and outer of said metal elements, and said filler elements of a plastic material characterized by flexibility and resiliency.

2. In a cable or rope, a strand comprising a central metal element, a ring of smaller diameter elements about said central element, a ring of metal elements about said ring of smaller diameter elements and of larger diameter, and said smaller diameter elements of a plastic material characterized by flexibility and resiliency.

3. In a cable or rope, a strand comprising inner and outer metal elements, said elements transversely circular and all of substantially the same diameter whereby in the assembled strand there are longitudinally extending spaces, and smaller diameter longitudinally extending filler elements in said spaces and tangentially engaging both the inner and outer of said metal elements, and said filler elements of polymerized vinylidene chloride.

4. In a cable or rope, a strand comprising a central metal element, a ring of smaller diameter elements about said central element, a ring of metal elements about said ring of smaller diameter elements and of larger diameter, and said smaller diameter elements of polymerized vinylidene chloride.

5. In a cable or rope, a strand comprising inner and outer metal elements, said elements transversely circular and all of substantially the same diameter whereby in the assembled strand there are longitudinally extending filler elements in said spaces and tangentially engaging both the inner and outer of said metal elements, said filler elements of a plastic material characterized by flexibility and resiliency, said metal and filler elements preformed into the spirals occupied by them in the rope, and said filler elements oriented along their spiral lines.

6. In a cable or rope, a strand comprising a central metal element, a ring of smaller diameter elements about said central element, a ring of metal elements about said ring of smaller diameter elements and of larger diameter, said smaller diameter elements of a plastic material characterized by flexibility and resiliency, the elements

of said rings preformed into the spirals occupied by them in the rope, and said elements of the plastic material oriented along said spirals.

7. A rope core comprising a single strand of layed rope of filaments of a synthetic plastic material having fibre forming characteristics, said filaments preformed into the spirals occupied by them in the core, and said filaments oriented spirally along the lines on which they are preformed.

8. A core or center for supporting the strands of a stranded wire rope, said core being formed of filament-like elements of a compound including a vinyl radical and having fibre forming characteristics, said elements being of substantially uniform cross-sectional area throughout their length whereby said core possesses a uniform bedding value, and each of said elements comprising a strip twisted upon itself and then while in such twisted state oriented by stretching.

9. In a wire rope, a core and a plurality of strands of wire layed helically about and radially supported by said core, said core comprising a smooth surfaced elongated body of a water-repellent synthetic chemical material immune to decay through biochemical attack, and said synthetic chemical material characterized by stretchability and by recovery when stretched whereby to stretch and not break on tensioning of the wire rope and to be capable of elongating and escaping into place from between wire strands of the rope when caught by said strands on bird caging of the rope.

10. In a wire rope, a core and a plurality of strands of wires layed helically about and radially supported by said core, said core comprising an elongated body of continuous, smooth surfaced filaments layed together, said filaments of a water-repellent synthetic chemical material immune to decay through biochemical attack, and said synthetic chemical material, when in filamentary form, characterized by stretchability and by recovery when stretched whereby to stretch and not break on tensioning of the wire rope and in such filamentary form capable of elongating and escaping into place from between wire rope strands when caught by them on bird caging of the rope.

11. In a cable, a primary core of a synthetic plastic material, wire ropes layed about said core, each of said ropes including a secondary core of a synthetic plastic material and a series of wires layed about and substantially covering said secondary core, each of said cores comprising continuous filaments of a water-repellent synthetic chemical material immune to decay through biochemical attack, said synthetic chemical material, when in filamentary form, characterized by flexibility and elasticity, said wire ropes and wires under tension about and deforming said cores, and said synthetic chemical material resilient whereby said cores are constantly tending to return to their normal conditions and thus fully support said wire ropes and said wires.

RICHARD F. WARREN, JR.